# EUROPEAN PATENT SPECIFICATION

(11) **EP 1 298 190 B1**
(45) Date of publication and mention of the grant of the patent: **12.10.2005**
(21) Application number: 02078107.6
(22) Date of filing: 30.07.2002
(51) Int. Cl.: C10M 163/00, C10N 10/12

(54) **Lubricating oil compositions for marine diesel engines**
Schmiermittelzusammensetzungen für Schiffsdieselmotoren
Compositions lubrifiantes pour la lubrification d'un moteur diesel marin

(30) Priority: 28.09.2001 EP 01308354
(43) Date of publication of application: 02.04.2003
(73) Proprietor: Infineum International Limited, Oxfordshire OX13 6BB (GB)
(72) Inventor: Chambard, Laurent, Faringdon, Oxfordshire SN7 8NQ (GB); Strickland, Keith, Didcot, Oxon OX11 9UY (GB)
(74) Representative: Lewis, Pauline Therese

(56) References cited:
- EP-A- 0 839 894
- EP-A- 1 087 008
- WO-A-96/20265
- US-A- 4 283 294
- US-A- 4 842 755
- US-A- 5 629 272
- US-A- 5 658 862
- US-A- 5 744 430
- US-A- 6 074 993
- US-A- 6 143 701
- US-B1- 6 277 794

## Description

The present invention concerns improved lubricating oil compositions for residual fuel oil-fuelled diesel engines. In particular, the present invention concerns lubricating oil compositions that demonstrate improved cylinder liner wear performance.

In large diesel engines of the cross-head type used in marine and heavy stationary applications, the cylinders are lubricated separately from the other engine components. The cylinders are lubricated on a total loss basis with the cylinder oil being injected separately to quills on each cylinder by means of lubricators positioned around the cylinder liner. Oil is distributed to the lubricators by means of pumps, which are, in modern engine designs, actuated to apply the oil directly onto the rings to reduce wastage of the oil. The high stresses encountered in these engines and the use of residual fuels creates the need for lubricants with a high detergency and neutralising capability even though the oils are exposed to thermal and other stresses only for short periods of time. Residual fuels commonly used in these diesel engines typically contain significant quantities of sulfur, which, in the combustion process, combine with water to form sulfuric acid, the presence of which leads to corrosive wear. In particular, in two-stroke engines for ships, areas around the cylinder liners and piston rings can be corroded and worn by the acid. Therefore, it is important for diesel engine lubricating oils to have the ability to resist such corrosion and wear.

The art describes the use of particular additives to neutralise the sulfuric acid formed and thus protect the cylinder liners and piston rings from corrosion and wear.

For example, US-A-4842755 discloses the use of borated dispersants and zinc dialkyldithiophosphates in a marine cylinder lubricating oil composition to provide anti-wear performance in the cylinder liner and piston ring areas.

US-A-4948522 discloses marine diesel cylinder lubricants comprising a borated dispersant and a polybutene, and optionally a zinc dialkyldithiophosphate and/or an overbased metal detergent. The lubricants have improved ring wear and linear wear performance and good protection against corrosion.

US-A-6140280 discloses succinimide compounds that exhibit corrosion resistance and wear resistance in diesel engines. It also discloses that conventional anti-wear agents, such as zinc dithiophosphates and molybdenum dithiocarbamates, may be used as co-additives.

WO 99/64543 discloses cylinder oils of defined characteristics and a liquid polyisobutylene. The cylinder oils provide improved performance including protection against corrosive, friction and abrasive wear.

The aim of the present invention is to provide a lubricating oil composition that offers effective cylinder liner protection, particularly in the areas of the cylinder that are prone to corrosive wear.

Accordingly, in a first aspect, the present invention provides a lubricating oil composition for a residual fuel oil-fuelled diesel engine for marine and stationary applications, comprising:
(a) an oil of lubricating viscosity, in a major amount;
(b) an oil-soluble or oil-dispersible trinuclear molybdenum compound, in a minor amount; and
(c) a detergent composition, which comprises one or more overbased metal detergents;
wherein the oil composition has a TBN from 30 to 100 as measured according to ASTM D-2896 and a viscosity at 100°C in the range from 9 to 30 mm² s⁻¹ as measured according to ASTM D-445.

In a second aspect, the present invention provides use of the lubricating oil composition in a cylinder of a two-stroke cross-head marine diesel engine, wherein the cylinder is characterised by a power output of 4000 or greater, such as 4200 or greater, preferably 4500 or greater, more preferably in the range of 4500 to 6000, kW.

In a third aspect, the present invention provides the use of an oil-soluble or oil-dispersible trinuclear molybdenum compound or a composition, such as an oleaginous composition, comprising the trinuclear molybdenum compound, to reduce corrosive wear in a cylinder liner of a residual fuel oil-fuelled diesel engine, preferably a cross-head marine engine.

In a fourth aspect, the present invention provides a method of reducing corrosive wear in a cylinder liner of a residual fuel oil-fuelled diesel engine, preferably a cross-head marine, comprising supplying to the walls of the cylinder a lubricating oil composition of the first aspect.

In a fifth aspect, the present invention provides an additive composition comprising:
(a) an oil-soluble or oil-dispersible trinuclear molybdenum compound;
(b) one or more co-additives; and
(c) a detergent composition, which comprises one or more overbased metal detergents;
wherein the additive composition contains (a) and (b) in an amount to provide a lubricating oil composition having a TBN from 30 to 100 as measured according to ASTM D-2896 and a viscosity at 100°C in the range from 9 to 30 mm² s⁻¹ as measured according to ASTM D-445, when the lubricating oil composition contains 5 to 40 mass % of the additive composition.

In this specification, the following words and expressions shall have the meanings ascribed below:
"major amount" means in excess of 50 mass % of the composition, preferably is excess of 60 mass %, more preferably in excess of 70 mass %, and most preferably in excess of 80 mass %;
"minor amount" means less that 50 mass % of the composition, preferably less than 40 mass %, more preferably less than 30 mass %, and most preferably less than 20 mass %, both in respect of the stated additive and in respect of the total mass % of all the additives present in the lubricant, reckoned as active ingredient of the additive or additives;
"active ingredient (a.i.)" refers to additive material that is not diluent or solvent.
"comprises or comprising" or cognate words specifies the presence of stated features, steps, integers or components, but does not preclude the presence or addition of one or more other features, steps, integers, components, or groups thereof;
"TBN" - Total Base Number as measured by ASTM D2896;
"oil-soluble or oil-dispersible" - does not necessarily indicate solubility, dissolvability, miscibility or capability of suppression in oil in all proportions. They do mean, however, solubility or stable dispersibility sufficient to exert the intended effect in the environment in which the oil is employed. Moreover, additional incorporation of other additives may permit incorporation of higher levels of a particular additive, if desired.

It will be understood that the various components of the lubricating oil composition, essential as well as optimal and customary, may react under the conditions of formulation, storage or use and that the invention also provides the product obtainable or obtained as a result of any such reaction.

The features of the invention will now be discussed in more detail below.

### Diesel Engines

Diesel fuel oils can in general be divided into two main categories - distillates and heavy or residual fuels. Distillates consist of one or more distillate fractions.

Heavy or residual fuels are fuels that comprise at least a proportion of a residual oil, i.e. oil that remains after the distilled fractions have been removed from unrefined oil. The composition of the residual fuel will vary with the composition of the starting oil, usually a crude oil, and will also vary depending upon the distillation conditions. However, by its nature, residual fuel oil is of high molecular weight, contains significant quantities of sulfur and has a high boiling point. The term "residual oil" is understood by those skilled in the art; it is defined according to the standards ISO 8217, ISO RME25 and ISO RME35.

The present invention is suitable for large residual fuel oil-fuelled diesel engines, such as diesel engines of the cross-head type used in marine and heavy stationary applications, and of the trunk piston type found in marine applications. Large diesel engines are mainly employed for marine propulsion and power generation. Diesel engines suitable in the present invention can also be fuelled by a mixture of distillate and residual fuels.

Cross-head engines tend to be two-stroke, whereas trunk piston engines tend to be four-stroke. Four-stroke trunk piston engines may have a speed of 100 to 2,000, preferably 300 to 1,800, more preferably 350 to 1500, rpm, and the cylinder is characterised by power output of 50 to 10000, preferably 100 to 6000, more preferably 150 to 5000, kW. Two-stroke cross-head engines may have a speed of 40 to 600, preferably 60 to 500, such as 80 to 300, rpm and the cylinder is characterised by a power output of 4000 or greater, such as 4200 or greater, preferably 4500 or greater, more preferably in the range of 4500 to 6000, kW. Further, the engines may, for example, have from 6 to 12 cylinders and their total output may, for example, be in the range of 18,000 to 70,000 kW. The bore of the cylinder may, for example, be 850 or greater, such as 900 or greater, preferably in the range of 900 to 1000, cm.

The lubricating oil compositions of the present invention are particularly useful in cross-head engines, such as two-stroke cross-head engines for marine propulsion and stationary power generation.

### Lubricating Oil Composition

In respect of each aspect of the present invention, the total base number (TBN) of the lubricating oil composition, independent of the viscosity at 100 °C, is preferably 30 to 95, more preferably 40 to 90, even more preferably 65 to 90.

In respect of each aspect of the present invention, the viscosity at 100 °C of the lubricating oil composition, independent of the TBN, is preferably 9 to 25, more preferably 12 to 25, even more preferably 16 to 25, such as 18 to 22, mm² s⁻¹.

In respect of each aspect of the present invention, the viscosity index, as defined by ASTM D2270, of the lubricating oil composition is preferably at least 90, more preferably at least 95, especially at least 100, for example in the range from 90 to 110.

Lubricating oil compositions used in large residual-fuelled diesel engines can become contaminated with residual fuel during use, particularly in four-stroke trunk piston engines. Therefore, the lubricating oil compositions of the invention can also contain a residual fuel oil.

The lubricating oil compositions of the present invention will typically be monograde, i.e. compositions that exhibit little or no viscosity index improvement properties, for example, an SAE30, SAE 40, SAE 50 or higher lubricant. Thus, lubricating oil compositions of the present invention preferably do not comprise a viscosity index modifier.

### Oil of Lubricating Viscosity

The oil of lubricating viscosity (sometimes referred to as lubricating oil) may be any oil suitable for the lubrication of a large diesel engine, such as a cross-head engine or a trunk piston engine. The lubricating oil may suitably be an animal, a vegetable or a mineral oil. Suitably the lubricating oil is a petroleum-derived lubricating oil, such as a naphthenic base, paraffinic base or mixed base oil. Alternatively, the lubricating oil may be a synthetic lubricating oil. Suitable synthetic lubricating oils include synthetic ester lubricating oils, which oils include diesters such as di-octyl adipate, di-octyl sebacate and tri-decyl adipate, or polymeric hydrocarbon lubricating oils, for example liquid polyisobutene and poly-alpha olefins. Commonly, a mineral oil is employed.

Another class of lubricating oils is hydrocracked oils, where the refining process further breaks down the middle and heavy distillate fractions in the presence of hydrogen at high temperatures and moderate pressures. Hydrocracked oils typically have kinematic viscosity at 100 °C of from 2 to 40, for example from 3 to 15, mm²s⁻¹ and a viscosity index typically in the range of from 100 to 110, for example from 105 to 108.

The term 'brightstock' as used herein refers to base oils which are solvent-extracted, de-asphalted products from vacuum residuum, which generally have a kinematic viscosity at 100 °C of from 28 to 36 mm²s⁻¹ and are typically used in a proportion of less than 30, preferably less than 20, more preferably less than 15, most preferably less than 10, such as less than 5, mass %, based on the mass of the lubricating oil composition.

### Trinuclear Molybdenum Compound

The lubricating oil compositions comprise an oil-soluble or oil-dispersible trinuclear molybdenum compound.

The trinuclear (or trimeric) molybdenum compounds are especially those of the formula Mo₃SₖLₙQ_{z} and mixtures thereof, wherein the L are independently selected ligands having organo groups with a sufficient number of carbon atoms to render the compound soluble in the oil, n is from 1 to 4, k varies from 4 to 7, Q is selected from the group of neutral electron donating compounds such as water, amines, alcohols, phosphines, and ethers, and z ranges from 0 to 5 and includes non-stoichiometric values. At least 21 total carbon atoms should be present among all the ligands' organo groups, such as at least 25, at least 30, or at least 35 carbon atoms.

The ligands may be selected from the group consisting of

-X-R 1,

and mixtures thereof, wherein X, X₁, X₂, and Y are selected from the group consisting of oxygen and sulfur, and wherein R₁, R₂, and R are selected from hydrogen and organo groups that may be the same or different. Preferably, the organo groups are hydrocarbyl groups such as alkyl (e.g., in which the carbon atom attached to the remainder of the ligand is primary or secondary), aryl, substituted aryl and ether groups. More preferably, each ligand has the same hydrocarbyl group.

The term "hydrocarbyl" as used herein denotes a substituent having carbon atoms directly attached to the remainder of the ligand and is predominantly hydrocarbyl in character. Such substituents include the following:
1. Hydrocarbon substituents, that is, aliphatic (for example alkyl or alkenyl), alicyclic (for example cycloalkyl or cycloalkenyl) substituents, aromatic-, aliphatic- and alicyclic-substituted aromatic nuclei, as well as cyclic substituents wherein the ring is completed through another portion of the ligand (that is, any two indicated substituents may together form an alicyclic group).
2. Substituted hydrocarbon substituents, that is, those containing non-hydrocarbon groups which do not alter the predominantly hydrocarbyl character of the substituent. Those skilled in the art will be aware of suitable groups (e.g., halo, especially chloro and fluoro, amino, alkoxyl, mercapto, alkylmercapto, nitro, nitroso, sulfoxy, etc.).

Importantly, the organo groups of the ligands have a sufficient number of carbon atoms to render the compound soluble in the oil. For example, the number of carbon atoms in each group will generally range between 1 to 100, preferably from 1 to 30, and more preferably between 4 to 20. Preferred ligands include dialkyldithiophosphate, alkylxanthate, carboxylates, dialkyldithiocarbamate ("dtc"), and mixtures thereof. Most preferred are the dialkyldithiocarbamates. Those skilled in the art will realize that formation of the compounds of the present invention requires selection of ligands having the appropriate charge to balance the core's charge (as discussed below).

Compounds having the formula Mo₃SₖLₙQ_{z} have cationic cores surrounded by anionic ligands, wherein the cationic cores are represented by structures such as which have net charges of +4. Consequently, in order to solubilize these cores the total charge among all the ligands must be -4. Four monoanionic ligands are preferred. Without wishing to be bound by any theory, it is believed that two or more trinuclear cores may be bound or interconnected by means of one or more ligands and the ligands may be multidentate, i.e., having multiple connections to one or more cores. It is believed that oxygen and/or selenium may be substituted for sulfur in the core(s).

Oil-soluble trinuclear molybdenum compounds can be prepared by reacting in the appropriate liquid(s)/solvent(s) a molybdenum source such as (NH₄)₂Mo₃S₁₃·n(H₂O), where n varies between 0 and 2 and includes non-stoichiometric values, with a suitable ligand source such as a tetralkylthiuram disulfide. Other oil-soluble trinuclear molybdenum compounds can be formed during a reaction in the appropriate solvent(s) of a molybdenum source such as (NH₄)₂Mo₃S₁₃·n(H₂O), a ligand source such as tetralkylthiuram disulfide, dialkyldithiocarbamate, or dialkyldithiophosphate, and a sulfur-abstracting agent such as cyanide ions, sulfite ions, or substituted phosphines. Alternatively, a trinuclear molybdenum-sulfur halide salt such as [M']₂[Mo₃S₇A₆], where M' is a counter ion, and A is a halogen such as Cl, Br, or I, may be reacted with a ligand source such as a dialkyldithiocarbamate or dialkyldithiophosphate in the appropriate liquid(s)/solvent(s) to form an oil-soluble trinuclear molybdenum compound. The appropriate liquid/solvent may be, for example, aqueous or organic.

The ligand chosen must have a sufficient number of carbon atoms to render the compound soluble in the lubricating composition.

Trinuclear molybdenum compounds for use in the compositions of this invention can be those of the formula Mo₃S₇((alkyl)₂dtc)₄ where the alkyl has about 8 to 18 carbon atoms. The alkyl is preferably a "coco" alkyl chain which is a mixture of chains of varying even numbers of carbon atoms from typically a C₈ to C₁₈ alkyl, mainly C₁₀, C₁₂ and C₁₄ alkyls derived from coconut oil.

Other examples of trinuclear molybdenum compounds include a sulfurized trinuclear molybdenum containing composition prepared by (i) reacting an acidic molybdenum compound and a basic nitrogen compound selected from the group consisting of succinimide, a carboxylic acid amide, a hydrocarbyl monoamine, a phosphoramide, a thiophosphoramide, a Mannich base, a dispersant viscosity index improver, or a mixture thereof, in the presence of a polar promoter, to form a trinuclear molybdenum complex, and (ii) reacting the trinuclear molybdenum complex with a sulfur-containing compound, to thereby form a sulfur- and molybdenum-containing composition.

In another embodiment of the present invention, the trinuclear molybdenum compound is preferably fully sulfurised, i.e. the core contains only sulfur, for example Mo₃S₄ and Mo₃S₇.

In another embodiment of the present invention, the trinuclear molybdenum compound is preferably a dithiocarbamate compound, such a trinuclear molybdenum dithiocarbamate; especially effective compounds are molybdenum dialkyldithiocarbamate compounds represented by the formula Mo₃S₇((alkyl)₂dtc)₄.

In each aspect the of present invention, the lubricating oil composition preferably contains 1 to 10000, more preferably 5 to 5000, even more preferably 10 to 1000, especially 50 to 750, ppm of molybdenum by mass, based on the mass of the oil composition.

Oil-soluble or oil-dispersible molybdenum compounds, such as trinuclear molybdenum dithiocarbamates, have been found to be particularly effective in preventing corrosive wear in the cylinder liner.

The amount of molybdenum is measured according to ASTM D5185.

### Dispersant

In respect of each aspect of the invention, the lubricating oil compositions can also comprise a dispersant. Dispersants maintain oil-insoluble substances, resulting from oxidation during use, in suspension in the fluid, thus preventing sludge flocculation and precipitation or deposition on metal parts.

So-called ashless dispersants are organic materials, which form substantially no ash on combustion, in contrast to metal-containing (and thus ash-forming) detergents. Borated metal-free dispersants are regarded herein as ashless dispersants.

Typically, the dispersants comprise amine, alcohol, amide, or ester polar moieties attached to the polymer backbone often via a bridging group. The dispersant may be, for example, selected from oil-soluble salts, esters, amino-esters, amides, imides, and oxazolines of long chain hydrocarbon substituted mono- and dicarboxylic acids or their anhydrides; thiocarboxylate derivatives of long chain hydrocarbons; long chain aliphatic hydrocarbons having a polyamine attached directly thereto; and Mannick condensation products formed by condensing a long chain substituted phenol with formaldehyde and polyalkylene polyamine, and Koch reaction products.

The polymer backbone is typically an olefin polymer, especially polymers comprising a major molar amount (i.e. greater than 50 mole %) of a C₂ to C₁₈ olefin (e.g., ethylene, propylene, butylene, isobutylene, pentene, octene-1, styrene), and typically a C₂ to C₅ olefin. The oil-soluble polymeric hydrocarbon backbone may be a homopolymer (e.g., polypropylene or polyisobutylene) or a copolymer of two or more of such olefins (e.g., copolymers of ethylene and an alpha-olefin such as propylene and butylene or copolymers of two different alphaolefins).

One preferred class of olefin polymers is polybutenes and specifically polyisobutenes (PIB) or poly-n-butenes, such as may be prepared by polymerization of a C₄ refinery stream. Another preferred class of olefin polymers is ethylene alpha-olefin (EAO) copolymers or alpha-olefin homo- and copolymers such as may be prepared using metallocene chemistry having in each case a high degree (e.g. >30%) of terminal vinylidene unsaturation.

The polymer backbone will usually have number average molecular weight ($\overline{\text{M}}$n) within the range of from 100 to 20,000 or 10,000. The $\overline{\text{M}}$n of the backbone is preferably within the range of 250 or 500 to 10,000, more preferably 700 to 5,000. Both relatively low molecular weight ($\overline{\text{M}}$n 500 to 1500) and relatively high molecular weight ($\overline{\text{M}}$n 1500 to 5,000 or greater) polymers are useful to make dispersants. Particularly useful olefin polymers for use in dispersants have $\overline{\text{M}}$n within the range of from 900 to 3000. The olefin polymers used to prepare dispersants preferably have approximately one terminal double bond per polymer chain.

Suitable dispersants include, for example, derivatives of long chain hydrocarbon-substituted carboxylic acids in which the hydrocarbon groups contain 50 to 400 carbon atoms, examples of such derivatives being derivatives of high molecular weight hydrocarbyl-substituted succinic acid. Such hydrocarbyl-substituted carboxylic acids may be reacted with, for example, a nitrogen-containing compound, advantageously a polyalkylene polyamine, or with an ester. Particularly preferred dispersants are the reaction products of polyalkylene amines with alkenyl succinic anhydrides. Examples of specifications disclosing dispersants of the last-mentioned type are US-A-3 202 678, 3 154 560, 3 172 892, 3 024 195, 3 024 237, 3 219 666, 3 216 936 and BE-A-662 875.

The dispersant can be further post-treated by a variety of conventional post treatments such as boration, as generally described in US 3,087,936 and 3,254,025. This is readily accomplished by treating an acyl nitrogen-containing dispersant with a boron compound selected from the group consisting of boron oxide, boron halides, boron acids and esters of boron acids or highly borated low $\overline{\text{M}}$w dispersant, in an amount to provide a boron to nitrogen mole ratio of 0.01 - 5.0. Usefully the dispersants contain from 0.05 to 2.0, e.g. 0.05 to 1.5 or 0.9, mass % of boron based on the total mass (active ingredient basis) of the borated acyl nitrogen compound.

Preferred for use in the invention is a polyisobutenyl succinimide dispersant wherein the $\overline{\text{M}}$n of the polyisobutenyl groups is from 750 to 3000, such as 900 to 1200 or 2000 to 2300.

In one embodiment of the present invention, the amount of dispersant, based on nitrogen derived from the dispersant, in the lubricating oil composition is preferably up to 1.0, more preferably 0.001 to 0.08, such as 0.005 to 0.55 or 0.50, mass %, based on the mass of the lubricating oil composition.

In another embodiment of the present invention, the amount of dispersant, based on boron derived from the dispersant, in the lubricating oil composition is preferably not more than 0.5, such as not more than 0.25, for example 0.005 to 0.1, mass %, based on the mass of the lubricating oil composition.

Preferably the dispersant is a borated dispersant, such as a borated succinimide.

The amount of boron is measured according to ASTM D5185; the amount of nitrogen is measured according to ASTM D5291; the $\overline{\text{M}}$n can be determined by several known techniques - a convenient method for such determination is by gel permeation chromatography (GPC) which additionally provides molecular weight distribution information.

### Detergent

In respect of each aspect of the invention, the lubricating oil composition comprises a detergent composition, which comprises one or more overbased detergents.

A detergent is an additive that reduces formation of piston deposits, for example high-temperature varnish and lacquer deposits, in engines; it has acid-neutralising properties and is capable of keeping finely divided solids in suspension. It is based on metal "soaps", that is metal salts of acidic organic compounds, sometimes referred to as surfactants.

Large amounts of a metal base can be included by reacting an excess of a metal compound, such as an oxide or hydroxide, with an acidic gas such as carbon dioxide to give an overbased detergent which comprises neutralised detergent as the outer layer of a metal base (e.g. carbonate) micelle.

The metals can be selected from Group 1 and Group 2 metals, e.g., sodium, potassium, lithium, calcium, and magnesium. Calcium and magnesium are preferred; more preferably the metal is calcium.

Surfactants that may be used include organic carboxylates, for example, aliphatic carboxylates and aromatic carboxylates, such as salicylates, non-sulfurised or sulfurised; sulfonates; phenates, non-sulfurised or sulfurised; thiophosphonates; and naphthenates.

Examples of suitable detergents include overbased metal phenates, metal sulfonates, metal salicylates and metal carboxylates, where the metal is selected from sodium, calcium and magnesium; preferably the metal is calcium.

Also suitable in each aspect of the present invention is a detergent in the form of a hybrid complex detergent, wherein the basic material is stabilised by more than one type of surfactant (see WO 97/46643, WO 97/46644, WO 97/46646, and WO 97/46647). It will be appreciated by one skilled in the art that a single type of organic acid may contain a mixture of organic acids of the same type. For example, a sulphonic acid may contain a mixture of sulphonic acids of varying molecular weights. Such an organic acid composition is considered as one type. Thus, complex detergents are distinguished from mixtures of two or more separate overbased detergents, an example of such a mixture being one of an overbased salicylate detergent with an overbased phenate detergent.

The art describes examples of overbased complex detergents. For example, International Patent Application Publication Nos. 9746643/4/5/6 and 7 describe hybrid complexes made by neutralising a mixture of more than one acidic organic compound with a basic metal compound, and then overbasing the mixture. Individual basic micelles of the detergent are thus stabilised by a plurality of surfactant types.

EP-A-0 750 659 describes a calcium salicylate phenate complex made by carboxylating a calcium phenate and then sulfurising and overbasing the mixture of calcium salicylate and calcium phenate. Such complexes may be referred to as "phenalates"

Surfactants for the surfactant system of the overbased metal detergent may contain at least one hydrocarbyl group, for example, as a substituent on an aromatic ring. Advantageously, hydrocarbyl groups in surfactants for use in accordance with the invention are aliphatic groups, preferably alkyl or alkylene groups, especially alkyl groups, which may be linear or branched. The total number of carbon atoms in the surfactants should be at least sufficient to impact the desired oil-solubility.

The proportion of one detergent type (e.g. calcium sulfonate) to another detergent type (e.g. sodium phenate) in the detergent composition is not critical. Similarly, the proportion of one surfactant to another in a complex detergent is not critical.

The detergent composition may comprise a major proportion of a phenate detergent or comprises a complex hybrid detergent having a major proportion of a phenate surfactant, where the phenate detergent or the complex hybrid detergent is preferably a calcium salt.

The overbased detergents of the present invention may have a TBN of at least 200, preferably at least 250, especially at least 300, such as up to 600.

The lubricating oil compositions of the present invention have a sufficient amount of additives, for example, detergents, whether neutral or overbased, to provide the required TBN. For example, the detergent composition may be used up to 30, preferably 2 to 15 or to 20, mass % of detergent composition, based on the mass of the lubricating oil composition.

### Co-Additives

The lubricants may include an antiwear agent as a co-additive and may also contain other co-additives, for example, antioxidants, antifoaming agents and/or rust inhibitors. Further details of particular co-additives are as follows.

Oxidation inhibitors, or antioxidants, reduce the tendency of mineral oils to deteriorate in service, evidence of such deterioration being, for example, the production of varnish-like deposits on metal surfaces and of sludge, and viscosity increase. Suitable oxidation inhibitors include sulphurized alkyl phenols and alkali or alkaline earth metal salts thereof; diphenylamines; phenyl-naphthylamines; and phosphosulphurized or sulphurized hydrocarbons.

Other oxidation inhibitors or antioxidants that may be used in the lubricant comprise oil-soluble copper compounds. The copper may be blended therein as any suitable oil-soluble copper compound. By oil-soluble is meant that the compound is oil-soluble under normal blending conditions in the base stock or an additive package. The copper may, for example, be in the form of a copper dihydrocarbyl thio- or dithio-phosphate. Alternatively, the copper may be added as the copper salt of a synthetic or natural carboxylic acid, for example, a C8 to C18 fatty acid, an unsaturated acid, or a branched carboxylic acid. Also useful are oil-soluble copper dithiocarbamates, sulphonates, phenates, and acetylacetonates. Examples of particularly useful copper compounds are basic, neutral or acidic copper Cu I and/or Cu II salts derived from alkenyl succinic acids or anhydrides.

Additional detergents and metal rust inhibitors include the metal salts, which may be overbased and have a TBN less than 300, of sulphonic acids, alkyl phenols, sulphurized alkyl phenols, alkyl salicylic acids, thiophosphonic acids, naphthenic acids, and other oil-soluble mono- and dicarboxylic acids. Representative examples of detergents/rust inhibitors, and their methods of preparation, are given in EP-A-208 560. In the case of metal salts of salicylic acids, the TBN of the metal salts may be less than 200.

Antiwear agents, as their name implies, reduce wear of metal parts. Zinc dihydrocarbyl dithiophosphates (ZDDPs) are very widely used as antiwear agents. Especially preferred ZDDPs are those of the formula Zn[SP(S)(OR₁)(OR₂)]₂ wherein R₁ and R₂ represent hydrocarbyl groups such as alkyl groups that contain from 1 to 18, preferably 2 to 12, carbon atoms. Also suitable are ashless or non-metal containing additives, such as sulfur and/or phosphorus containing compounds, for example, sulfurised phenol and amine dithiophosphate.

The oil compositions of the present invention may contain 0 to 0.2, preferably 0.05 to 0.15, more preferably 0.01 to 0.1, mass % of phosphorus, based on the mass of the oil composition. In a preferred embodiment of the present invention, the oil composition contains less than 150, preferably less than 100, more preferably less than 50, for example 0, ppm of phosphorus.

Pour point depressants, otherwise known as lube oil flow improvers, lower the minimum temperature at which the fluid will flow or can be poured. Such additives are well known. Foam control may be provided by an antifoamant of the polysiloxane type, for example, silicone oil or polydimethyl siloxane.

Typical proportions for additives for a four-stroke trunk piston engine oil composition are as follows:

| **Additive** | **Mass % a.i.*** **(Broad)** | **Mass % a.i.*** **(Preferred)** |
|---|---|---|
| Detergent(s) | 0.5-10 | 2-7 |
| Dispersant(s) | 0.5-5 | 1-3 |
| Anti-wear agent(s) | 0.1-1.5 | 0.5-1.3 |
| Oxidation inhibitor | 0.2-2 | 0.5-1.5 |
| Rust inhibitor | 0.03-0.15 | 0.05-0.1 |
| Pour point depressant | 0.03-0.15 | 0.05-0.1 |
| Mineral or synthetic base oil | Balance | Balance |

| | | |
|---|---|---|
| * Mass % active ingredient based on the final oil composition. | | |

Typical proportions for additives for a two-stroke cross-head oil composition are as follows:

| **Additive** | **Mass % a.i.*** **(Broad)** | **Mass % a.i.* (Preferred)** |
|---|---|---|
| Detergent(s) | 1-18 | 3-12 |
| Dispersant(s) | 0.5-5 | 1-3 |
| Anti-wear agent(s) | 0.1-1.5 | 0.5-1.3 |
| Pour point depressant | 0.03-0.15 | 0.05-0.1 |
| Mineral or synthetic base oil | Balance | Balance |

| | | |
|---|---|---|
| * Mass % active ingredient based on the final oil composition. | | |

When a plurality of additives is employed it may be desirable, although not essential, to prepare one or more additive compositions (also known as packages) or concentrates comprising the additives, whereby several additives can be added simultaneously to the oil of lubricating viscosity to form the lubricant or lubricating oil composition. Dissolution of the additive package(s) into the oil of lubricating viscosity may be facilitated by solvents and by mixing accompanied with mild heating, but this is not essential. The additive package(s) will typically be formulated to contain the additive(s) in proper amounts to provide the desired concentration, and/or to carry out the intended function, in the final lubricant when the additive package(s) is/are combined with a predetermined amount of oil of lubricating viscosity.

Thus, the molybdenum compound in accordance with the present invention may be admixed with small amounts of base oil or other compatible solvents together with other desirable additives to form additive packages containing active ingredients in an amount, based on the additive package, of, for example, from 2.5 to 90 and preferably from 5 to 75 and most preferably from 8 to 60, mass %, the remainder being base oil or other compatible solvents.

The lubricating oil composition may typically contain 5 to 40, preferably 10 to 38, more preferably 16 to 34, mass % of the additive package(s), based on active ingredient.

The present invention is illustrated by, but in no way limited to, the following examples.

### Examples

Lubricating oil compositions were prepared by methods known in the art. Table 1 shows the compositional details of Example 1 and Comparative Examples 1 and 2. Example 1 and Comparative Examples 1 & 2 were blended so that the resulting lubricating oil composition has a TBN of 70 and viscosity at 100°C of about 20 mm²s⁻¹.

Example 1, an example according to the present invention, is a lubricating oil composition comprising 550 ppm of molybdenum; Comparative Examples 1 and 2 contain the same detergents and dispersant as Example 1, but Comparative Example 1 contains a zinc dithiophosphate additive instead of the molybdenum compound and Comparative Example 2 does not contain the molybdenum compound or the zinc compound. Comparative Example 3 is a commercial lubricating oil composition having a TBN of 70 and viscosity at 100°C of about 20 mm²s⁻¹.

The lubricating oil compositions of Example 1 and Comparative Examples 1 to 3 were tested for cylinder liner wear performance in a slow speed two-stroke cross-head "Bolnes" engine. Such engines are widely used by those skilled in the art for lubricating performance evaluation such as disclosed in a presentation by Nippon Mitsubishi Oil Company on 10 May 2001 at CIMAC conference entitled "The influence of the neutralisation ability of marine lubricants on engine lubrication" Takeshmia et al.

The cylinder liner wear data for Example 1 and Comparative Examples 1 to 3 are provided in Table 2. The data shows that Example 1 provides better wear protection than any one of Comparative Examples 1 to 3, in particular better than Comparative Example 1, which contains ZDDP. This improvement is especially evident in positions 2 to 5 of the cylinder.

## Claims

1. A lubricating oil composition for a residual fuel oil-fuelled diesel engine for marine and stationary applications, comprising:
(a) an oil of lubricating viscosity, in a major amount;
(b) an oil soluble or oil-dispersible trinuclear molybdenum compound, in a minor amount; and
(c) a detergent composition, which comprises one or more overbased metal detergents;
wherein the oil composition has a TBN from 30 to 100 as measured according to ASTM D-2896 and a viscosity at 100°C in the range from 9 to 30 mm²s⁻¹ as measured according to ASTM D-445.

2. The lubricating oil composition as claimed.in any one of the preceding claims, in the form of a residual-fuelled cross-head marine diesel engine lubricating oil composition having a TBN from 30 to 95 and a viscosity at 100°C in the range from 9 to 25, such as 12 to 25, mm²s⁻¹.

3. The lubricating oil composition as claimed in any one of the preceding claims, further comprising:
(d) a dispersant, which has a hydrocarbon backbone of molecular weight from 100 to 10000.

4. The lubricating oil composition as claimed in any one of the preceding claims, wherein the molybdenum compound is present in an amount from 1 to 10000 ppm of molybdenum by mass, based on the mass of the oil composition.

5. The lubricating oil composition as claimed in any one of the preceding claims, further comprising a residual fuel oil.

6. Use of the lubricating oil composition as claimed in any one of the preceding claims , in a two-stroke cross-head marine diesel engine wherein the cylinder is **characterised by** a power output of 4000 or greater, such as 4200 or greater, preferably 4500 or greater, more preferably in the range of 4500 to 6000, kW.

7. Use of an oil-soluble or oil-dispersible trinuclear molybdenum compound or a composition comprising the trinuclear molybdenum compound to reduce corrosive wear in a cylinder liner of a residual fuel oil-fuelled diesel engine.

8. A method of reducing corrosive wear in a cylinder liner of a residual fuel oil-fuelled diesel engine comprising supplying to the walls of the cylinder a lubricating oil composition as claimed in any one of claims 1 to 5.

9. An additive composition comprising:
(a) an oil-soluble or oil-dispersible trinuclear molybdenum compound;
(b) one or more co-additives; and
(c) a detergent composition, which comprises one or more overbased metal detergents;
wherein the additive composition contains (a) and (b) in an amount to provide a lubricating oil composition having a TBN from 30 to 100 as measured according to ASTM D-2896 and a viscosity at 100°C in the range from 9 to 30 mm²s⁻¹ as measured according to ASTM D-445, when the lubricating oil composition contains 5 to 40 mass % of the additive composition.

## Patentansprüche

1. Schmierölzusammensetzung für einen mit Rückstandsbrennstofföl betriebenen Dieselmotor für Schiffe und stationäre Anwendungen, die:
(a) ein Öl mit Schmierviskosität in einer größeren Menge,
(b) eine in Öl lösliche oder in Öl dispergierbare dreikernige Molybdänverbindung in einer geringeren Menge und
(c) eine Detergenszusammensetzung umfasst, die ein oder mehrere überbasische Metalldetergentien umfasst,
wobei die Ölzusammensetzung eine TBN von 30 bis 100, gemessen gemäß ASTM D-2896, und eine Viskosität bei 100 °C im Bereich von 9 bis 30 mm²s⁻¹, gemessen gemäß ASTM D-445, aufweist.

2. Schmierölzusammensetzung nach einem der vorhergehenden Ansprüche in Form einer Schmierölzusammensetzung für einen mit Rückstandbrennstoff betriebenen Kreuzkopfschiffsdieselmotor mit einer TBN von 30 bis 95 und einer Viskosität bei 100 °C im Bereich von 9 bis 25, wie beispielsweise 10 bis 25 mm²s⁻¹.

3. Schmierölzusammensetzung nach einem der vorhergehenden Ansprüche, die ferner
(d) ein Dispergiermittel umfasst, das ein Kohlenwasserstoffgerüst mit einem Molekulargewicht von 100 bis 10 000 aufweist.

4. Schmierölzusammensetzung nach einem der vorhergehenden Ansprüche, bei dem die Molybdänverbindung in einer Gewichtsmenge von 1 bis 10 000 ppm Molybdän bezogen auf das Gewicht der Ölzusammensetzung vorhanden ist.

5. Schmierölzusammensetzung nach einem der vorhergehenden Ansprüche, die ferner Rückstandsbrennstofföl umfasst.

6. Verwendung einer Schmierölzusammensetzung gemäß einem der vorhergehenden Ansprüche in einem Zweitaktkreuzkopfschiffsdieselmotor, bei dem der Zylinder durch eine Leistungsabgabe von 4000 oder größer, wie beispielsweise 4200 oder größer, bevorzugt 4500 oder größer, bevorzugter im Bereich von 4000 bis 6000 kw **gekennzeichnet** ist.

7. Verwendung einer in Öl löslichen oder in Öl dispergierbaren, dreikernigen Molybdänverbindung oder einer Zusammensetzung, die die dreikernige Molybdänverbindung umfasst, zur Verringerung von Korrosionsverschleiß in einer Zylinderbüchse eines mit Rückstandsbrennstofföl betriebenen Dieselmotors.

8. Verfahren zur Verringerung von Korrosionsverschleiß in einer Zylinderbüchse eines mit Rückstandsbrennstofföl betriebenen Dieselmotors, bei dem den Wänden des Zylinders eine Schmierölzusammensetzung gemäß einem der Ansprüche 1 bis 5 zugeführt wird.

9. Additivzusammensetzung, die:
(a) eine in Öl lösliche oder in Öl dispergierbare, dreikernige Molybdänverbindung,
(b) ein oder mehrere Co-Additive und
(c) eine Detergenszusammensetzung umfasst, die ein oder mehrere überbasische Metalldetergentien umfasst,
wobei die Additivzusammensetzung (a) und (b) in einer Menge enthält, um eine Schmierölzusammensetzung mit einer TBN von 30 bis 100, gemessen gemäß ASTM D-2896, und einer Viskosität bei 100 °C im Bereich von 9 bis 30 mm²s⁻¹, gemessen gemäß ASTM D-445, zu liefern, wenn die Schmierölzusammensetzung 5 bis 40 Mass.-% der Additivzusammensetzung enthält.

## Revendications

1. Composition d'huile lubrifiante pour un moteur Diesel alimenté en huile combustible résiduelle pour des applications marines et fixes, comprenant :
(a) une huile ayant une viscosité lubrifiante en une quantité principale ;
(b) un composé trinucléaire du molybdène soluble dans l'huile ou dispersable dans l'huile en une petite quantité ; et
(c) une composition de détergent comprenant un ou plusieurs détergents à base de métaux surbasifiés ;
ladite composition d'huile ayant un indice de basicité totale (TBN) de 30 à 100, mesuré conformément à ASTM D-2896, et une viscosité à 100°C dans la plage de 9 à 30 mm²s⁻¹, mesurée conformément à ASTM D-445.

2. Composition d'huile lubrifiante selon l'une quelconque des revendications précédentes, sous la forme d'une composition d'huile lubrifiante pour un moteur Diesel marin 'à crosse alimenté en huile combustible résiduelle, ayant une valeur de TBN de 30 à 95 et une viscosité à 100°C dans la plage de 9 à 25, par exemple de 12 à 25 mm²s⁻¹.

3. Composition d'huile lubrifiante selon l'une quelconque des revendications précédentes, comprenant en outre :
(d) un dispersant qui a un squelette d'hydrocarbure ayant un poids moléculaire de 100 à 10 000.

4. Composition d'huile lubrifiante selon l'une quelconque des revendications précédentes, dans laquelle le composé du molybdène est présent en une quantité de 1 à 10 000 ppm en poids de molybdène par rapport au poids de la composition d'huile.

5. Composition d'huile lubrifiante selon l'une quelconque des revendications précédentes, comprenant en outre une huile combustible résiduelle.

6. Utilisation de la composition d'huile lubrifiante selon l'une quelconque des revendications précédentes dans un moteur Diesel marin à crosse à deux temps dans lequel le cylindre est **caractérisé par** une puissance utile de 4000 ou plus, par exemple de 4200 ou plus, de préférence de 4500 ou plus, de façon plus préférée dans la plage de 4500 à 6000 kW.

7. Utilisation d'un composé trinucléaire du molybdène soluble dans l'huile ou dispersable dans l'huile ou d'une composition comprenant le composé trinucléaire du molybdène pour réduire l'usure par corrosion dans une chemise de cylindre d'un moteur Diesel alimenté en huile combustible résiduelle.

8. Procédé pour réduire l'usure par corrosion dans une chemise de cylindre d'un moteur Diesel alimenté en huile combustible résiduelle, comprenant l'amenée sur les parois du cylindre d'une composition d'huile lubrifiante selon l'une quelconque des revendications 1 à 5.

9. Composition d'additifs comprenant :
(a) un composé trinucléaire du molybdène soluble dans l'huile ou dispersable dans l'huile ;
(b) un ou plusieurs co-additifs ; et
(c) une composition de détergent comprenant un ou plusieurs détergents à base de métaux surbasifiés ;
ladite composition d'additifs contenant (a) et (b) en une quantité fournissant une composition d'huile lubrifiante ayant une valeur de TBN de 30 à 100, mesurée conformément à ASTM D-2896, et une viscosité à 100°C dans la plage de 9 à 30 mm²s⁻¹, mesurée conformément à ASTM D-445, quand la composition d'huile lubrifiante contient de 5 à 40 % en poids de la composition d'additifs.
